



US010260136B2

(12) **United States Patent**  
**Yoon**

(10) **Patent No.:** **US 10,260,136 B2**  
(45) **Date of Patent:** **Apr. 16, 2019**

(54) **ALUMINUM ALLOY FOR DIE CASTING AND METHOD OF HEAT TREATING THE SAME**

(71) Applicant: **Hyundai Motor Company**, Seoul (KR)

(72) Inventor: **Hyung Sop Yoon**, Gyeonggi-do (KR)

(73) Assignee: **Hyundai Motor Company**, Seoul (KR)

(\*) Notice: Subject to any disclaimer, the term of this patent is extended or adjusted under 35 U.S.C. 154(b) by 281 days.

(21) Appl. No.: **15/278,668**

(22) Filed: **Sep. 28, 2016**

(65) **Prior Publication Data**

US 2017/0314111 A1 Nov. 2, 2017

(30) **Foreign Application Priority Data**

Apr. 27, 2016 (KR) ..... 10-2016-0051200

(51) **Int. Cl.**

**C22F 1/043** (2006.01)

**C22C 21/02** (2006.01)

**B22D 18/06** (2006.01)

**B22D 21/00** (2006.01)

(52) **U.S. Cl.**

CPC ..... **C22F 1/043** (2013.01); **B22D 18/06**

(2013.01); **B22D 21/007** (2013.01); **C22C**

**21/02** (2013.01)

(58) **Field of Classification Search**

None

See application file for complete search history.

(56) **References Cited**

U.S. PATENT DOCUMENTS

7,625,454 B2 12/2009 Lin et al.  
2002/0053373 A1\* 5/2002 Feikus ..... C22F 1/043  
148/417

|                  |        |                |                        |
|------------------|--------|----------------|------------------------|
| 2003/0041934 A1* | 3/2003 | Lumley .....   | C22F 1/04<br>148/698   |
| 2003/0047250 A1* | 3/2003 | Takasaki ..... | C22F 1/043<br>420/532  |
| 2003/0143102 A1* | 7/2003 | Matsuoka ..... | C22F 1/043<br>420/532  |
| 2005/0076977 A1* | 4/2005 | Lumley .....   | C22F 1/043<br>148/698  |
| 2009/0038720 A1* | 2/2009 | Lumley .....   | C22C 21/02<br>148/695  |
| 2010/0224293 A1* | 9/2010 | Wang .....     | C22C 21/02<br>148/701  |
| 2013/0186525 A1* | 7/2013 | Koch .....     | B22D 21/007<br>148/549 |

FOREIGN PATENT DOCUMENTS

|    |                |   |         |
|----|----------------|---|---------|
| GB | 2128205 A      | * | 4/1984  |
| JP | 05/179384      | * | 7/1993  |
| JP | H05179384 A    |   | 7/1993  |
| JP | 2008-514807 A  |   | 5/2008  |
| JP | 2009-024265 A  |   | 2/2009  |
| KR | 2002-0077184 A |   | 10/2002 |
| KR | 10-0648487 B1  |   | 11/2006 |
| KR | 2014-0091858 A |   | 7/2014  |
| KR | 10-1571665 B1  |   | 11/2015 |
| WO | 2006/014948 A2 |   | 2/2006  |

OTHER PUBLICATIONS

English translation of JP 05/179384, Jul. 1993; 7 pages.\*

\* cited by examiner

Primary Examiner — Helene Klemanski

(74) Attorney, Agent, or Firm — Mintz Levin Cohn Ferris Glovsky and Popeo, P.C.; Peter F. Corless

(57) **ABSTRACT**

Disclosed are an aluminum alloy composition for die casting and a method of heat treating the same. The aluminum alloy composition contains precipitation of an Mg—Zn-based strengthening phase through heat treatment to thus enhance strength thereof.

**17 Claims, 14 Drawing Sheets**



FIG. 1



FIG. 2



FIG. 3



FIG. 4



FIG. 5



FIG. 6



FIG. 7



FIG. 8



FIG. 9



FIG. 10



FIG. 11



FIG. 12



FIG. 13



FIG. 14

**ALUMINUM ALLOY FOR DIE CASTING  
AND METHOD OF HEAT TREATING THE  
SAME**

**CROSS REFERENCE TO RELATED  
APPLICATION**

The present application claims priority to Korean Patent Application No. 10-2016-0051200, filed Apr. 27, 2016, the entire contents of which is incorporated herein for all purposes by this reference.

**TECHNICAL FIELD**

The present invention relates to an aluminum alloy composition that may be suitable for die casting and a method of heat treating the same. In particular, the aluminum alloy composition may include precipitation of an Mg—Zn-based strengthening phase formed by heat treatment and thus may have substantially improved strength thereof.

**BACKGROUND OF THE INVENTION**

As being easily cast, being efficiently alloyed with other metals, exhibiting high corrosion resistance in air, and having high electrical and thermal conductivities, aluminum has been widely utilized in industry.

In particular, aluminum has been mostly used to reduce the weight of vehicles and to increase fuel efficiency, and has been provided in the form of an aluminum alloy, by mixing aluminum with other metals, because the strength of aluminum itself may not be sufficient as compared to the other metals such as iron.

The aluminum alloy has been manufactured by die-casting, which is a precision casting process in which a molten metal is injected into a mold having a cavity that is mechanically processed at high precision in accordance with the shape of the product to be cast, thus obtaining a cast product having the same shape as that of the cavity.

Meanwhile, the aluminum alloy for die casting has to possess properties suitable for use in a process of filling the cavity of the mold with a high-speed high-pressure molten metal within a short time (for example, within 0.1 to 0.3 sec) to solidify it. In particular, appropriate high-temperature viscosity and latent heat may be required, thereby ensuring flowability suitable for high-pressure casting and mitigating shrinkage defects upon solidification.

Examples of aluminum alloys that have been known for use in die casting include ADC10 alloy that contains an amount of about 8 to 12 wt % of silicon (Si) to thus show properties suitable for the die-casting process and A380 alloy that contains an amount of about 2 to 4 wt % of copper (Cu) to ensure the strength required of structural material even without additional heat treatment.

The ADC10 and A380 alloys also include iron (Fe) in a maximum amount of about 1.3 wt % in order to minimally inhibit seizure and corrosion between the aluminum melt and the mold. Typically, side effects including low elongation due to an excess of Fe acicular structure are minimized through structural fineness using quenching, thus enabling the recycling of the alloy, thereby increasing productivity and work convenience.

The ADC10 and A380 alloys may constitute 90% or greater of all alloys for die casting, because of the many advantages thereof, including their properties and high productivity.

When a die-casting process is commonly applied, no heat treatment has been known to be carried out. Recently, however, many attempts have been made to increase alloy strength using high-vacuum die-casting techniques or heat treatment techniques having a short solution treatment time.

The foregoing is intended merely to aid in the understanding of the background of the present invention, and is not intended to mean that the present invention falls within the purview of the related art that is already known to those skilled in the art.

**SUMMARY OF THE INVENTION**

In preferred aspects, the present invention provides an aluminum alloy composition that may be suitably used for die casting and a method of heat treating the same. In particular, the method of heat treating the aluminum alloy composition of the present invention suitably may form precipitation of a Zn-based strengthening phase, instead of a conventional Cu-based strengthening phase, thereby improving strength through heat treatment.

In one aspect of the present invention, provided is an aluminum alloy composition for die casting. The aluminum alloy composition may comprise: silicon (Si) in an amount of about 9.6 to 12.0 wt %; magnesium (Mg) in an amount of about 1.5 to 3.0 wt %; zinc (Zn) in an amount of about 3.0 to 6.0 wt %; iron (Fe) in an amount of about 1.3 wt % or less but greater than 0 wt %; manganese (Mn) in an amount of about 0.5 wt % or less but greater than 0 wt %; nickel (Ni) in an amount of about 0.5 wt % or less but greater than 0 wt %; tin (Sn) in an amount of about 0.2 wt % or less but greater than 0 wt %; and aluminum (Al) constituting the remaining balance of the aluminum alloy composition. Unless otherwise indicated herein, all the wt % are based on the total weight of the aluminum alloy composition.

The aluminum alloy may further include copper (Cu) in an amount of about 0.3 wt % or less, based on the total weight of the aluminum alloy composition. In addition, the aluminum alloy may further include titanium (Ti) in an amount of about 0.3 wt % or less, based on the total weight of the aluminum alloy composition. The aluminum alloy may further include copper (Cu) in an amount of about 0.3 wt % or less and titanium (Ti) in an amount of about 0.3 wt % or less, based on the total weight of the aluminum alloy composition.

Preferably, the sum of amounts of Mg and Zn may be of about 6 to 8 wt %, based on the total weight of the aluminum alloy composition.

Preferably, the aluminum alloy composition may have a ratio of Mg/Zn ratio about 2.0 or greater.

The aluminum alloy suitably may have a yield strength of about 300 MPa or greater.

The aluminum alloy suitably may have a tensile strength of about 350 MPa or greater.

The aluminum alloy suitably may have an elongation of about 2% or greater.

Further provided is the aluminum alloy composition that may consist essentially of, essentially consist of or consist of the components as described herein. For example, the aluminum alloy composition that may consist essentially of, essentially consist of or consist of: silicon (Si) in an amount of about 9.6 to 12.0 wt %; magnesium (Mg) in an amount of about 1.5 to 3.0 wt %; zinc (Zn) in an amount of about 3.0 to 6.0 wt %; iron (Fe) in an amount of about 1.3 wt % or less but greater than 0 wt %; manganese (Mn) in an amount of about 0.5 wt % or less but greater than 0 wt %; nickel (Ni) in an amount of about 0.5 wt % or less but greater than 0 wt %

%; tin (Sn) in an amount of about 0.2 wt % or less but greater than 0 wt %; and aluminum (Al) constituting the remaining balance of the aluminum alloy composition.

The aluminum alloy also may consist essentially of, essentially consist of or consist of silicon (Si) in an amount of about 9.6 to 12.0 wt %; magnesium (Mg) in an amount of about 1.5 to 3.0 wt %; zinc (Zn) in an amount of about 3.0 to 6.0 wt %; iron (Fe) in an amount of about 1.3 wt % or less but greater than 0 wt %; manganese (Mn) in an amount of about 0.5 wt % or less but greater than 0 wt %; nickel (Ni) in an amount of about 0.5 wt % or less but greater than 0 wt %; tin (Sn) in an amount of about 0.2 wt % or less but greater than 0 wt %; copper (Cu) in an amount of about 0.3 wt % or less; and aluminum (Al) constituting the remaining balance of the aluminum alloy composition.

In addition, the aluminum alloy also may consist essentially of, essentially consist of or consist of silicon (Si) in an amount of about 9.6 to 12.0 wt %; magnesium (Mg) in an amount of about 1.5 to 3.0 wt %; zinc (Zn) in an amount of about 3.0 to 6.0 wt %; iron (Fe) in an amount of about 1.3 wt % or less but greater than 0 wt %; manganese (Mn) in an amount of about 0.5 wt % or less but greater than 0 wt %; nickel (Ni) in an amount of about 0.5 wt % or less but greater than 0 wt %; tin (Sn) in an amount of about 0.2 wt % or less but greater than 0 wt %; titanium (Ti) in an amount of about 0.3 wt % or less; and aluminum (Al) constituting the remaining balance of the aluminum alloy composition.

In another aspect, provided is a method of heat treating an aluminum alloy composition for die casting. The method may comprise: preparing, by a solution treatment, a solution-treated aluminum alloy from an aluminum alloy composition that may be manufactured by die casting; primary aging the solution-treated aluminum alloy so as to form an  $MgZn_2$  precipitate; and secondary aging the aluminum alloy having the  $MgZn_2$  precipitate so as to form an  $Mg_2Si$  precipitate.

The term "solution treatment" as used herein, refers to a heating or heat treating an alloy and alloy components thereof, which is followed by a rapid cooling to hold the alloy components in a form of a solid solution, in which a portion the alloy components can be uniformly distributed and mixed within the crystal lattice of the major component. For example, during the solution treatment, the aluminum alloy of the present application may be partially melt and some minor components may be in a dissolved state or uniformly distributed state in aluminum component.

The primary aging suitably may be performed at a temperature of about 110 to 130° C. for about 10 to 24 hours.

The secondary aging suitably may be performed at a temperature of about 160 to 180° C. for about 3 to 6 hours.

The aluminum alloy may include: silicon (Si) in an amount of about 9.6 to 12.0 wt %; magnesium (Mg) in an amount of about 1.5 to 3.0 wt %; zinc (Zn) in an amount of about 3.0 to 6.0 wt %; iron (Fe) in an amount of about 1.3 wt % or less but greater than 0 wt %; manganese (Mn) in an amount of about 0.5 wt % or less but greater than 0 wt %; nickel (Ni) in an amount of about 0.5 wt % or less but greater than 0 wt %; tin (Sn) in an amount of about 0.2 wt % or less but greater than 0 wt %; copper (Cu) in an amount of about 0.3 wt % or less; and aluminum (Al) constituting the remaining balance of the aluminum alloy composition.

In addition, the aluminum alloy further comprises at least one from copper (Cu) in an amount of about 0.3 wt % or less and tin (Ti) in an amount of about 0.3 wt % or less, based on the total weight of the aluminum alloy.

Still provided is a vehicle that may comprise the aluminum alloy composition as described herein.

Other aspects of the present invention are disclosed infra.

According to various exemplary embodiments of the present invention, the inclusion of Cu may be maximally inhibited, the amounts of Mg and Zn may be optimally set, and heat treatment conditions may be optimized so as to be adapted for an alloy composition, thus increasing strength while ensuring castability similar to that of conventional ADC10 and A380 alloys.

Also, castability equal to or greater than the conventional ADC10 and A380 alloys may be obtained, conventional molds and systems may be applied without change, and the production yield may be maintained at the same level.

In addition, the effects of impurities such as Fe on the properties of the alloy may be reduced such that the alloy may be recyclable.

#### BRIEF DESCRIPTION OF THE DRAWINGS

The above and other features and advantages of the present invention will be more clearly understood from the following detailed description taken in conjunction with the accompanying drawings, in which:

FIG. 1 illustrates results of differential scanning calorimetry (DSC) of precipitates that are formed when an A380 alloy is added with Zn in amounts of 1, 2 and 3 wt %;

FIG. 2 illustrates the results of analysis of the properties of an A380 alloy when added with Zn in amounts of 1, 2 and 3 wt %;

FIG. 3 illustrates results of phase analysis of an ADC12 alloy (Al-2.5Cu-0.15Mg-10.5Si-0.5Zn);

FIG. 4 illustrates results of phase analysis of an ADC12 alloy (Al-2.5Cu-1.0Fe-2.0Mg-10.5Si-4.5Zn);

FIG. 5 illustrates results of phase analysis of an A7075 alloy (Al-2.5Cu-2.0Mg-1.0Si-6.0Zn);

FIG. 6 illustrates results of phase analysis of an A7075 alloy (Al-2.5Cu-2.0Mg-5.0Si-6.0Zn);

FIG. 7 illustrates results of phase analysis of an A380 alloy (Al-2.5Cu-2.0Mg-10.5Si-4.5Zn);

FIG. 8 illustrates results of phase analysis of the A380 alloy (Al-2.5Cu-2.0Mg-10.5Si-6.0Zn);

FIG. 9 illustrates test results of an exemplary Al—Cu—Mg—Si—Zn alloy according to an exemplary embodiment of the present invention depending on changes in the amount of Si;

FIG. 10 illustrates results of phase analysis for producing a heat-treatment strengthening phase (Al—Cu—Mg—Si);

FIG. 11 illustrates results of phase analysis of an exemplary alloy according to an exemplary embodiment of the present invention depending on the amount of Cu; and

FIG. 12 illustrates results of phase analysis of an exemplary alloy according to an exemplary embodiment of the present invention depending on the amount of Cu;

FIG. 13 illustrates changes in the strengthening phase attributable to Mg depending on the amount of Cu in an exemplary alloy (Al-2.5Cu-1.0Fe-2.0Mg-10.5Si-4.5Zn) of the present invention; and

FIG. 14 illustrates changes in the strengthening phase attributable to Mg depending on the amount of Cu in an exemplary alloy (Al-1.0Cu-1.0Fe-2.0Mg-0.3Mn-10.5Si-3.5Zn) of the present invention.

#### DESCRIPTION OF SPECIFIC EMBODIMENTS

The terminology used herein is for the purpose of describing particular exemplary embodiments only and is not intended to be limiting of the invention. As used herein, the singular forms "a", "an" and "the" are intended to include

the plural forms as well, unless the context clearly indicates otherwise. It will be further understood that the terms "comprises" and/or "comprising," when used in this specification, specify the presence of stated features, integers, steps, operations, elements, and/or components, but do not preclude the presence or addition of one or more other features, integers, steps, operations, elements, components, and/or groups thereof. As used herein, the term "and/or" includes any and all combinations of one or more of the associated listed items.

Unless specifically stated or obvious from context, as used herein, the term "about" is understood as within a range of normal tolerance in the art, for example within 2 standard deviations of the mean. "About" can be understood as within 10%, 9%, 8%, 7%, 6%, 5%, 4%, 3%, 2%, 1%, 0.5%, 0.1%, 0.05%, or 0.01% of the stated value. Unless otherwise clear from the context, all numerical values provided herein are modified by the term "about."

It is understood that the term "vehicle" or "vehicular" or other similar term as used herein is inclusive of motor vehicles in general such as passenger automobiles including sports utility vehicles (SUV), buses, trucks, various commercial vehicles, watercraft including a variety of boats and ships, aircraft, and the like, and includes hybrid vehicles, electric vehicles, plug-in hybrid electric vehicles, hydrogen-powered vehicles and other alternative fuel vehicles (e.g. fuels derived from resources other than petroleum). As referred to herein, a hybrid vehicle is a vehicle that has two or more sources of power, for example both gasoline-powered and electric-powered vehicles.

Hereinafter, a detailed description will be given of embodiments of the present invention with reference to the appended drawings. However, the present invention is not limited to the following embodiments, which may be changed in various embodiments. These embodiments are provided to complete the disclosure of the present invention, and to fully describe the present invention to those skilled in the art.

According to the present invention, an aluminum alloy for die casting suitably may include a precipitation strengthening phase to improve strength through heat treatment for high-pressure die casting while retaining the advantages of conventional ADC10 and A380 alloys.

In order to obtain the alloy characteristics required for a die-casting process according to the present invention, the amounts of iron (Fe), manganese (Mn), nickel (Ni), tin (Sn), and titanium (Ti) may be maintained similar to those of corresponding components in the conventional ADC10 alloy or A380 alloy, and the amounts of other alloy components may be suitably adjusted to maximize the precipitation strengthening effect. Particularly, in the exemplary aluminum alloys of the present invention, silicon (Si), copper (Cu), magnesium (Mg) and zinc (Zn) may be main components used for improving strength by precipitation thereof, and may be formed into precipitates such as  $Al_2Cu$ ,  $Mg_2Si$  and  $MgZn_2$ .

For example, according to an exemplary embodiment of the present invention, the aluminum alloy for die casting may comprise silicon (Si) in an amount of about 9.6 to 12.0 wt %; magnesium (Mg) in an amount of about 1.5 to 3.0 wt %; zinc (Zn) in an amount of about 3.0 to 6.0 wt %; iron (Fe) in an amount of about 1.3 wt % or less but greater than 0 wt %; manganese (Mn) in an amount of about 0.5 wt % or less but greater than 0 wt %; nickel (Ni) in an amount of about 0.5 wt % or less but greater than 0 wt %; tin (Sn) in an amount of about 0.2 wt % or less but greater than 0 wt %; and aluminum (Al) constituting the remaining balance of the

aluminum alloy composition. In order to improve the heat treatment effect, preferably, an amount of about 0.3 wt % or less of Ti may be further included. Alternatively, an amount of Cu, which may be inevitably mixed therewith, may be included but limited to about 0.3 wt % or less.

In the present invention, the reason why the alloy components and the amounts thereof are limited is as follows. Unless otherwise stated, "%", when representing the unit of the amount of the component, refers to "wt %".

10 Silicon (Si) suitably may be included in an amount of about 9.6 to 12.0%. Si as used herein may improve castability and form a precipitate, such that the Si content may be included in the maximum amount at a temperature equal to or less than a eutectic point. Accordingly, the amount of Si 15 suitably may range from about 9.6% to about 12.0%.

Magnesium (Mg) suitably may be included in an amount of about 1.5 to 3.0%. Mg may form a precipitate, however, when added greater than the predetermined amount, for example, greater than about 3.0%, castability and properties 20 may deteriorate and inclusions may be generated due to oxidation. Accordingly, the amount of Mg suitably may range from about 1.5% to about 3.0%.

Zinc (Zn) suitably may be included in an amount of about 3.0 to 6.0%. Zn as used herein may form precipitate of 25 strengthening phase that may replace a Cu-based strengthening phase in the present invention, and thus a Zn—Mg-based strengthening phase may be precipitated.

In particular, the amount of copper (Cu) may be limited to about 0.3% or less. Typically, Cu in an aluminum alloy for 30 die casting may be used as a precipitation strengthening element, and thus plays a role in strengthening the aluminum alloy. Accordingly, the alloy may be designed so as to include Cu in an amount of about 4.0% which is the solid solution limit. The simple addition of Cu in an amount equal 35 to or greater than the solid solution limit in order to increase the heat-treatment strengthening effect may cause problems since Cu may not be dissolved in Al and thus there may not be sufficient improvement to the properties, and side effects may occur due to segregation. Accordingly, since the 40 strength of the alloy cannot be increased as desired by the use of the Cu-based strengthening phase, Cu suitably may be included in a minimum amount required to precipitate a Zn-based strengthening phase. Cu may be inevitably mixed upon forming the aluminum alloy, and thus the amount 45 thereof may be limited to about 1% or less, and preferably about 0.3% or less.

In addition, a method of heat treating the aluminum alloy for die casting according to an exemplary embodiment of the present invention is suitable for heat treatment of the alloy 50 having the above components in the above amounts, the method may include: preparing, by a solution treatment, a solution-treated aluminum alloy from an aluminum alloy that may be manufactured through die casting; primary aging the solution-treated aluminum alloy so as to form a 55  $MgZn_2$  precipitate; and secondary aging the aluminum alloy having the  $MgZn_2$  precipitate so as to form an  $Mg_2Si$  precipitate.

Preferably, the primary aging may be performed at a 60 temperature of about 110 to 130° C. for about 10 to 24 hours, and the secondary aging may be performed at a temperature of about 160 to 180° C. for about 3 to 6 hours.

The reason why the amounts of silicon (Si), copper (Cu), magnesium (Mg) and zinc (Zn) may be limited and the reason why the aging process may be limited are described 65 below.

In the present embodiment, in order to increase the strength of the alloy as desired while decreasing the amount

of Cu compared to the ADC10 and A380 alloys, heat treatment for  $MgZn_2$ , which is an Mg—Zn-based strengthening phase, was performed, and the amounts of Mg and Zn in the conventional A380 alloy were adjusted.

#### TEST EXAMPLE 1

The precipitates resulting from adding the A380 alloy with Zn in amounts of 1, 2 and 3% were analyzed using DSC. The results are illustrated in FIG. 1 and the following Table 1.

As illustrated in FIG. 1 and Table 1,  $Al_2Cu$  and  $Mg_2Si$  precipitates were observed when Zn was added in an amount of 1%, but no Zn phase was observed. Even when Zn was added in an amount of 3%, the Zn phase was not observed, and the  $Mg_2Si$  phase was decreased (the dotted line A). These results are deemed to be because the amount of dissolved Mg is decreased due to the solid solution of excess Zn or because an additional composite appears in lieu of  $Mg_2Si$ .

TABLE 1

| Intermediate precipitate | Phase appearance | Measurement | Heat flow (mW/g)    |         |         |
|--------------------------|------------------|-------------|---------------------|---------|---------|
|                          |                  |             | Temp. on DSC (° C.) | 1 wt. % | 2 wt. % |
| $\theta''(Al_2Cu)$       |                  | 140~150     | 147                 | 63      | 42      |
| $\theta'(Al_2Cu)$        |                  | 170~190     | 170                 | 82      | 71      |
| $\beta''(Mg_2Si)$        |                  | 230~250     | 241                 | 61      | 55      |
| $\eta''(MgZn_2)$         |                  | 250~260     | —                   | —       | 21      |
|                          |                  |             |                     | No peak |         |

Thus, the strengthening effect could not be obtained through the simple addition of Zn. Also, the addition of Zn resulted in a reduction in  $Mg_2Si$ , which is a conventional strengthening phase, rather than the production of the desired  $MgZn_2$  precipitate.

In addition, the properties of the A380 alloy were analyzed when added with Zn in amounts of 1, and 2 and 3%. The results are illustrated in FIG. 2.

As shown in FIG. 2, strength (hardness) was not increased as desired when Zn was added. When the amount of Zn was greater than 2%, hardness was decreased slightly. Accordingly, when Zn is present in a solid solution phase, and thus when the dissolved amount thereof is increased, the dissolved amounts of other alloying elements may be decreased.

The reason why Zn is not present in the form of the  $MgZn_2$  precipitate is that Mg, existing in a relatively small amount, may be consumed to thus produce  $Mg_2Si$  upon solidification in the presence of Si. In this case, when Mg is provided in a sufficient amount, the  $Mg_2Si$  phase may be oversaturated and that the remaining amount thereof may be formed into an  $MgZn_2$  phase.

Under this assumption, even when the amounts of both Zn and Mg were increased, heat treatment properties were not improved as desired.

#### TEST EXAMPLE 2

In order to determine the reason why desired heat treatment properties were not obtained despite the increase in the amounts of Zn and Mg in Test Example 1, phase analysis programs were performed. The conventional ADC12 alloy was phase analyzed. The results are illustrated in FIGS. 3 and 4.

FIG. 3 illustrates the results of phase analysis when Fe is not added, and FIG. 4 illustrates the results of phase analysis when Fe is added.

As illustrated in FIG. 3, the strengthening phase upon heat treatment of ADC12 was mainly considered to be  $Al_2Cu$ . Furthermore, the precipitate began to be formed at a temperature of about 460° C., which indicated that  $Al_2Cu$  was dissolved under conventionally known solution treatment conditions of a temperature of 480 to 520° C. The formation of the Mg strengthening phase was hindered due to the production of a composite in the presence of Cu and Si. As shown in FIG. 4, in the presence of Fe, the Mg strengthening phase was formed into a composite through the reaction with Fe, making it difficult to attain heat treatment effects even in the case of die casting products to be quenched.

Therefore, when the amounts of both Zn and Mg are increased, the strength may be improved due to  $Al_2Cu$  and strength may be increased upon heat treatment. In the case of  $Mg_2Si$ , another strengthening phase, it was formed into a  $Si—Cu—Mg$  composite and was consumed by a Fe composite, making it difficult to contribute to an increase in strength upon heat treatment. Also, Mg was consumed even by the Fe—Mg—Si composite, which corresponds to the results of evaluating the actual optimal aging temperature. Therefore, the strength appeared to be maximally increased at a temperature of 160 to 180° C., corresponding to the aging temperature of the Cu phase.

#### TEST EXAMPLE 3

The results of phase analysis of the A7075 alloy, which is a typical  $MgZn_2$  alloy, are illustrated in FIGS. 5 and 6.

FIG. 5 illustrates the results of phase analysis of the A7075 alloy, and FIG. 6 illustrates the results of addition of excess Si to the casting material.

The A7075 alloy was produced in the sequence of  $Mg_2Si \rightarrow Al_2Cu \rightarrow MgZn_2 \rightarrow Al—Cu—Mg—Si$  composite, and the  $MgZn_2$  phase was produced in the greatest amount. When excess Si was added, no strengthening phases other than  $Al_2Cu$  was formed, and Zn was present only in a solid solution phase, because the  $Si—Cu—Mg$  composite appears upon addition of excess Si.

#### TEST EXAMPLE 4

The results of phase analysis of the alloys developed by adding the conventional A380 alloy with Zn and Mg are illustrated in FIGS. 7 and 8.

FIG. 7 illustrates the results of addition of 4.5% of Zn, and FIG. 8 illustrates the results of addition of 6.0% of Zn.

Like Test Example 2,  $Mg_2Si$  was consumed after the appearance of the composite ( $Al_5Cu_2Mg_8Si_6$ ), and  $Al_2Cu$  began to be produced at a temperature of 400° C. or less. The resultant Zn\_HCP may be a solid solution phase, and  $MgZn_2$  may not be formed.

Thus, when Zn and Mg were excessively added, the  $MgZn_2$  strengthening phase of interest was not formed, and only the solid solution phase was formed, which matches the results of evaluation of the precipitates using DSC. The addition of the A380 alloy with Zn is unsuitable for enhancing the strength, which may be due to appearance of the  $Si—Cu—Mg$  composite ( $Al_5Cu_2Mg_8Si_6$ ) in the presence of Si, as shown in the results of phase analysis of the A7075 alloy.

In order to develop the Zn-based die casting alloy for heat treatment, it may be essential to inhibit the production of the composite  $Al_5Cu_2Mg_8Si_6$ . This composite was produced at

a temperature of about 500° C., and was known to be formed together with Al<sub>2</sub>Cu. Hence, it may be important to inhibit the production of the composite through the control of the alloy components, rather than heat treatment conditions.

Thus, in the present invention, the production of the composite may be inhibited by removing any one of the composite elements.

#### TEST EXAMPLE 5

In order to evaluate changes in the other compounds depending on the amount of Si, the amount of Si in the Al-2.5Cu-2.0Mg-(Si)-5.0Zn alloy was changed. The results of phase analysis are illustrated in FIG. 9.

As illustrated in FIG. 9, when the amount of Si was 1% or greater, the composite (Al<sub>5</sub>Cu<sub>2</sub>Mg<sub>8</sub>Si<sub>6</sub>) appeared. When the amount of Si was 1.85% or greater, Mg and Cu were consumed to thus produce the composite (Al<sub>5</sub>Cu<sub>2</sub>Mg<sub>8</sub>Si<sub>6</sub>), rather than the formation of Mg<sub>2</sub>Si and Al<sub>2</sub>Cu. Based on the above results, Si may essentially be contained in a predetermined amount in the casting alloy, and thus, production of the composite may be inhibited through the control of the Si component.

Also, Mg may be the component of the main strengthening phase in the present invention, and thus, minimizing the amount of Cu, which is the remaining component, may be considered as appropriate in order to inhibit the production of the composite.

#### TEST EXAMPLE 6

FIG. 10 illustrates the results of phase analysis in the Cu-free alloy, containing Si in the same amount as in the ADC12 alloy and Zn and Mg in respective amounts of 4.5 and 2.0 wt %, in order to form the heat-treatment strengthening phase (Al—Cu—Mg—Si).

As illustrated in FIG. 10, MgZn<sub>2</sub> and Mg<sub>2</sub>Si were produced in large amounts, and Zn was not dissolved, but was present only in a precipitation strengthening phase. Furthermore, MgZn<sub>2</sub> was present in a stable phase at a temperature of about 130° C.

The alloy was configured to include Fe because another composite Al—Fe—Si—Mg was likely to result. Based on the analysis results, however, since the composite had a stable phase only at a temperature of 400° C. or greater, the amount of Mg that was consumed was not large upon actual die casting.

#### TEST EXAMPLE 7

The results of phase analysis when Cu is added in amounts of 1% and 2% are illustrated in FIGS. 11 and 12.

FIG. 11 illustrates the results of addition of 1% of Cu, and FIG. 13 illustrates the results of addition of 2% of Cu.

As shown in FIG. 12, when the amount of Cu was added in an amount of 1%, the Al<sub>5</sub>Cu<sub>2</sub>Mg<sub>8</sub>Si<sub>6</sub> composite was shown in a predetermined amount (less than 5%), and MgZn<sub>2</sub> was present in a stable phase, and some solid solution phase appeared.

As shown in FIG. 12, when the amount of Cu was 2%, the Al<sub>5</sub>Cu<sub>2</sub>Mg<sub>8</sub>Si<sub>6</sub> composite was produced in an amount of 6% or greater, and the MgZn<sub>2</sub> phase was not produced. Accordingly, the amount of Cu in the developed alloy may be limited to 1% or less.

#### TEST EXAMPLE 8

By comparing the amounts of Mg distributed in each alloy, whether any phase was produced by Mg was analyzed. The results are illustrated in FIGS. 13 and 14.

As illustrated in FIG. 13, when Cu was present in an amount of 2.0 wt % or greater, Mg was consumed only to produce the Al—Cu—Mg—Si composite and the strengthening phases were not present, and Zn was present in a solid solution phase.

As illustrated in FIG. 14, when Cu was present in an amount of 1%, Mg was partially consumed to thus produce an Al—Cu—Mg—Si composite, but contributed to the formation of strengthening phases, and the Zn solid solution phase was not readily apparent.

The components and amounts of the conventional alloys for die casting and the alloy for die casting according to Example of the present invention are compared and shown in Table 2 below.

TABLE 2

|    | Alloy   | Si   | Cu  | Mg  | Zn  | Fe  | Mn  | Ni  | Sn   | Ti  |
|----|---------|------|-----|-----|-----|-----|-----|-----|------|-----|
| 20 | ADC10   | min. | 7.5 | 2   | —   | —   | —   | —   | —    | —   |
|    |         | max. | 9.5 | 4   | 0.3 | 1   | 1.3 | 0.5 | 0.2  | 0.3 |
| 25 | ADC12   | min. | 9.6 | 1.5 | —   | —   | —   | —   | —    | —   |
|    |         | max. | 12  | 3.5 | 0.3 | 1   | 1.3 | 0.5 | 0.2  | 0.3 |
| 30 | A380    | min. | 7.5 | 3   | —   | —   | —   | —   | —    | —   |
|    |         | max. | 9.5 | 4   | 0.1 | 3   | 1.3 | 0.5 | 0.35 | —   |
| 35 | A7075   | min. | —   | 1.2 | 2.1 | 5.1 | —   | —   | —    | —   |
|    |         | max. | 0.4 | 2   | 2.9 | 6.1 | 0.5 | 0.3 | —    | 0.2 |
| 40 | Example | min. | 9.6 | —   | 1.5 | 3   | —   | —   | —    | —   |
|    |         | max. | 12  | 0.3 | 3   | 6   | 1.3 | 0.5 | 0.2  | 0.3 |

The alloy of Example was composed of Zn and Mg in amounts of 3.0 to 6.0% and 1.5 to 3.0%, respectively, in order to enhance strength. As such, to inhibit the formation of the composite that hinders the production of the main strengthening phases MgZn<sub>2</sub> and Mg<sub>2</sub>Si, the amount of Cu was limited to 0.3% or less, and, to maximize heat treatment effects, a fining agent Ti was added in an amount of 0.1 to 0.5%.

Furthermore, in order to ensure castability for die casting, the amount of Si was maximally ensured at a eutectic point or less, and the amount of Fe was maintained the same as in conventional alloys.

The properties of the alloy may be determined by the amount of Zn+Mg. When the amount of Zn+Mg is about 9% or greater, strength and heat treatment effects may be maximized, but also, stress corrosion may increase and casting moldability may be decreased. On the other hand, when the amount of Zn+Mg is within a range of about 6 to 8%, high strength may be maintained and side effects such as corrosion, molding, and the like may be reduced. Accordingly, these components are used in the above amount range. As such, when the Zn/Mg ratio is 2.0 or greater, MgZn<sub>2</sub> may be suitably formed. In the case where the Zn/Mg ratio is less than the above value, Mg<sub>3</sub>Zn<sub>3</sub>Al<sub>2</sub> is formed. Accordingly, the Zn/Mg ratio in the developed alloy may be at about 2.0 or greater.

Iron (Fe) does not cause properties to significantly decrease when the amount thereof is about 1.3% or less, corresponding to the typical recycling alloy level, and thus, the level of the impurities may be controlled in conventional typical die casting alloy, together with Mn and Sn.

Meanwhile, the two strengthening phases that were produced may have different temperatures at which individual precipitates are produced, such that maximum strength upon heat treatment under the same conditions may not be sufficiently obtained. In the present embodiment, MgZn<sub>2</sub>, having a low precipitation temperature, was first precipitated, and

## 11

then  $Mg_2Si$  was formed, whereby individual precipitates were precipitated maximally in the form of a coherent phase in order to increase strength.

In the primary aging step, the temperature may be maintained in the range of about 110 to 130° C. for about 10 to 24 hours, corresponding to typical 7000 series aluminum alloy conditions, and secondary aging may be performed at a temperature of about 160 to 180° C. for 3 to 6 hours. Upon primary aging, the precipitated  $MgZn_2$  may be converted into an incoherent phase that is stable under secondary aging temperature conditions. When the secondary aging time is greater than the predetermined time, for example, greater than about 6 hours, the properties may deteriorate. Also, during the primary aging, some  $Mg_2Si$  may be precipitated, and thus the secondary aging time may be preferably controlled to be less than a typical level.

The properties of the alloys according to the present embodiment were evaluated as follows.

Using aluminum alloys having the following compositions of Table 3, tensile samples were manufactured using a high-vacuum die casting system and then subjected to solution treatment at about 500° C. or greater for 6 hours or greater in order to maximize the aging temperature, after which primary aging was performed at a temperature of about 120° C. for 12 hours to precipitate  $MgZn_2$  and secondary aging was conducted at 175° C. for 3 hours to precipitate  $Mg_2Si$ . The properties of the manufactured samples were evaluated. The results are shown in Table 4 below.

TABLE 3

| Component (wt %) | Si   | Cu   | Mg   | Zn   | Fe   | Mn   | Ti  |
|------------------|------|------|------|------|------|------|-----|
| #1               | 10.5 | 0.24 | 2.02 | 4.1  | 0.88 | 0.35 | —   |
| #2               | 10.1 | 0.22 | 1.98 | 4.08 | 0.78 | 0.35 | 0.2 |

TABLE 4

| No.   | YS (MPa) | UTS (MPa) | EL (%) |
|-------|----------|-----------|--------|
| #1    | 332      | 416       | 2.93   |
| #2    | 336      | 415       | 3.13   |
| ADC12 | 170      | 250       | 1.2    |

As shown in Table 3, compared to conventional ADC12, yield strength was increased about two times, and tensile strength was increased about 1.6 times, and further, elongation was increased about 2.5 times.

Using Sample #1, the properties of alloys were tested under heat treatment conditions. The heat treatment conditions and results are shown in Table 5 below.

TABLE 5

| Type | Heat treatment conditions |                    | Tensile        |                |               |
|------|---------------------------|--------------------|----------------|----------------|---------------|
|      | Solution treatment        | Aging              | Strength (MPa) | Elongation (%) | Hardness (HB) |
| T6   | 500° C. 6 hours           | 110° C. 12 hours + | 395            | 2.51           | 120           |
|      | 520° C. 6 hours           | 180° C. 3 hours    | 424            | 2.98           | 118           |
|      | 500° C. 4 hours           |                    | 398            | 1.49           | 115           |
|      | 520° C. 4 hours           |                    | 421            | 2.56           | 118           |
| T5   | 530° C. 6 hours           | 110° C. 10 hours + | 401            | 3.01           | 113           |
|      |                           | 180° C. 6 hours    |                |                |               |
|      |                           | 110° C. 10 hours + | 426            | 2.36           | 125           |
|      |                           | 180° C. 3 hours    |                |                |               |

## 12

TABLE 5-continued

| Type | Heat treatment conditions |                    | Tensile        |                |               |
|------|---------------------------|--------------------|----------------|----------------|---------------|
|      | Solution treatment        | Aging              | Strength (MPa) | Elongation (%) | Hardness (HB) |
|      |                           | 120° C. 20 hours + | 411            | 1.78           | 122           |
|      |                           | 160° C. 6 hours    |                |                |               |
|      |                           | 120° C. 20 hours + | 412            | 2.31           | 119           |
|      |                           | 160° C. 3 hours    |                |                |               |

10

As shown in Table 5, the longer the primary aging time, the lower the secondary aging effects. The maximum properties were exhibited under aging conditions at a temperature of 110° C. for 10 hours followed by a condition at a temperature of 180° C. for 3 hours. Thus, heat treatment conditions may suitably be applied according to the end use within the temperature and time ranges of primary aging and secondary aging.

Although the various exemplary embodiments of the present invention have been disclosed for illustrative purposes, those skilled in the art will appreciate that various modifications, additions and substitutions are possible, without departing from the scope and spirit of the invention as disclosed in the accompanying claims.

What is claimed is:

1. An aluminum alloy composition, comprising: silicon (Si) in an amount of about 9.6 to 12.0 wt %; magnesium (Mg) in an amount of about 1.5 to 3.0 wt %; zinc (Zn) in an amount of about 3.0 to 6.0 wt %; iron (Fe) in an amount of about 1.3 wt % or less but greater than 0 wt %; manganese (Mn) in an amount of about 0.5 wt % or less but greater than 0 wt %; nickel (Ni) in an amount of about 0.5 wt % or less but greater than 0 wt %; tin (Sn) in an amount of about 0.2 wt % or less but greater than 0 wt %; and aluminum (Al) constituting the remaining balance of the aluminum alloy composition, all the wt % based on the total weight of the aluminum alloy composition, wherein a sum of amounts of Mg and Zn is of about 6 to 8 wt %.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7

## 13

9. The aluminum alloy composition of claim 1, consisting essentially of:  
 silicon (Si) in an amount of about 9.6 to 12.0 wt %;  
 magnesium (Mg) in an amount of about 1.5 to 3.0 wt %;  
 zinc (Zn) in an amount of about 3.0 to 6.0 wt %;  
 iron (Fe) in an amount of about 1.3 wt % or less but greater than 0 wt %;  
 manganese (Mn) in an amount of about 0.5 wt % or less but greater than 0 wt %;  
 nickel (Ni) in an amount of about 0.5 wt % or less but greater than 0 wt %;  
 tin (Sn) in an amount of about 0.2 wt % or less but greater than 0 wt %; and  
 aluminum (Al) constituting the remaining balance of the aluminum alloy composition,  
 all the wt % based on the total weight of the aluminum alloy composition.

10. The aluminum alloy composition of claim 1, consisting essentially of:  
 silicon (Si) in an amount of about 9.6 to 12.0 wt %;  
 magnesium (Mg) in an amount of about 1.5 to 3.0 wt %;  
 zinc (Zn) in an amount of about 3.0 to 6.0 wt %;  
 iron (Fe) in an amount of about 1.3 wt % or less but greater than 0 wt %;  
 manganese (Mn) in an amount of about 0.5 wt % or less but greater than 0 wt %;  
 nickel (Ni) in an amount of about 0.5 wt % or less but greater than 0 wt %;  
 tin (Sn) in an amount of about 0.2 wt % or less but greater than 0 wt %;  
 copper (Cu) in an amount of about 0.3 wt % or less and aluminum (Al) constituting the remaining balance of the aluminum alloy composition,  
 all the wt % based on the total weight of the aluminum alloy composition.

11. The aluminum alloy composition of claim 1, consisting essentially of:  
 silicon (Si) in an amount of about 9.6 to 12.0 wt %;  
 magnesium (Mg) in an amount of about 1.5 to 3.0 wt %;  
 zinc (Zn) in an amount of about 3.0 to 6.0 wt %;  
 iron (Fe) in an amount of about 1.3 wt % or less but greater than 0 wt %;  
 manganese (Mn) in an amount of about 0.5 wt % or less but greater than 0 wt %;  
 nickel (Ni) in an amount of about 0.5 wt % or less but greater than 0 wt %;  
 tin (Sn) in an amount of about 0.2 wt % or less but greater than 0 wt %;  
 titanium (Ti) in an amount of about 0.3 wt % or less; and aluminum (Al) constituting the remaining balance of the aluminum alloy composition,  
 all the wt % based on the total weight of the aluminum alloy composition.

12. The aluminum alloy composition of claim 1, consisting essentially of:  
 silicon (Si) in an amount of about 9.6 to 12.0 wt %;  
 magnesium (Mg) in an amount of about 1.5 to 3.0 wt %;

## 14

zinc (Zn) in an amount of about 3.0 to 6.0 wt %;  
 iron (Fe) in an amount of about 1.3 wt % or less but greater than 0 wt %;  
 manganese (Mn) in an amount of about 0.5 wt % or less but greater than 0 wt %;  
 nickel (Ni) in an amount of about 0.5 wt % or less but greater than 0 wt %;  
 tin (Sn) in an amount of about 0.2 wt % or less but greater than 0 wt %;  
 copper (Cu) in an amount of about 0.3 wt % or less;  
 titanium (Ti) in an amount of about 0.3 wt % or less; and aluminum (Al) constituting the remaining balance of the aluminum alloy composition,  
 all the wt % based on the total weight of the aluminum alloy composition.

13. A method of heat treating an aluminum alloy for die casting, comprising:

preparing, by a solution treatment, a solution-treated aluminum alloy from an aluminum alloy that is manufactured via die casting;  
 primary aging the solution-treated aluminum alloy so as to form an  $MgZn_2$  precipitate; and  
 secondary aging the aluminum alloy containing the  $MgZn_2$  precipitate so as to form an  $Mg_2Si$  precipitate, wherein the aluminum alloy comprise:  
 silicon (Si) in an amount of about 9.6 to 12.0 wt %;  
 magnesium (Mg) in an amount of about 1.5 to 3.0 wt %;  
 zinc (Zn) in an amount of about 3.0 to 6.0 wt %;  
 iron (Fe) in an amount of about 1.3 wt % or less but greater than 0 wt %;  
 manganese (Mn) in an amount of about 0.5 wt % or less but greater than 0 wt %;  
 nickel (Ni) in an amount of about 0.5 wt % or less but greater than 0 wt %;  
 tin (Sn) in an amount of about 0.2 wt % or less but greater than 0 wt %; and  
 aluminum (Al) constituting the remaining balance of the aluminum alloy composition,  
 all the wt % based on the total weight of the aluminum alloy composition,  
 wherein a sum of amounts of Mg and Zn is of about 6 to 8 wt %.

14. The method of claim 13, wherein the primary aging is performed at a temperature of about 110 to 130° C. for about 10 to 24 hours.

15. The method of claim 13, wherein the secondary aging is performed at a temperature of about 160 to 180° C. for about 3 to 6 hours.

16. The method of claim 13, wherein the aluminum alloy further comprises at least one from copper (Cu) in an amount of about 0.3 wt % or less and tin (Ti) in an amount of about 0.3 wt % or less, based on the total weight of the aluminum alloy.

17. A vehicle comprising an aluminum alloy composition of claim 1.

\* \* \* \* \*